# EUROPEAN PATENT SPECIFICATION

(11) **EP 3 894 613 B1**
(45) Date of publication and mention of the grant of the patent: **24.01.2024**
(21) Application number: 18913203.8
(22) Date of filing: 13.12.2018
(51) Int. Cl.: C23C 18/12

(54) **A ZEOLITE COATING PREPARATION ASSEMBLY AND METHOD FOR OPERATING THE SAME**
ZEOLITHBESCHICHTUNGSVORBEREITUNGSANORDNUNG UND VERFAHREN ZUM BETRIEB DAVON
ENSEMBLE DE PRÉPARATION DE REVÊTEMENT DE ZÉOLITE ET SON PROCÉDÉ DE FONCTIONNEMENT

(43) Date of publication of application: 20.10.2021
(73) Proprietor: Erdem, Ayse, Sariyer 34450 Istanbul (TR); Tatlier, Melkon, Sisli 34371 Istanbul (TR); Maras, Taylan, Kagithane 34415 Istanbul (TR)
(72) Inventor: Erdem, Ayse, Sariyer 34450 Istanbul (TR); Tatlier, Melkon, Sisli 34371 Istanbul (TR); Maras, Taylan, Kagithane 34415 Istanbul (TR)
(74) Representative: Atalay, Baris
(86) International application number: PCT/TR2018/050804
(87) International publication number: WO 2020/122826

(56) References cited:
- EP-A2- 2 820 170
- US-A- 3 202 537
- US-A- 3 529 989
- US-A- 3 652 322
- XU X ET AL: "SYNTHESIS OF A HIGH-PERMEANCE NAA ZEOLITE MEMBRANE BY MICROWAVE HEATING", ADVANCED MATERIALS, WILEY-VCH GERMANY, DE, vol. 12, no. 3, 3 February 2000 (2000-02-03), pages 195-198, XP000923551, ISSN: 0935-9648, DOI: 10.1002/(SICI)1521-4095(200002)12:3<195::A ID-ADMA195>3.0.CO;2-E cited in the application

## Description

### Technical Field of the Present Invention

The present invention relates to a zeolite coating preparation assembly and operation method where zeolite adsorbents are coated through a crystallization process on surfaces with the method of heating by induction.

### Background of the Present Invention

Zeolites are microporous crystalline aluminosilicates. Zeolite-like materials such as aluminophosphates (AlPOs), silicoaluminophosphates (SAPOs), metal aluminophosphates (MeAPOs), and metal silicoaluminophosphates (MeSAPOs), etc., are also known to exist and have recently been considered by many in the literature as belonging to the family of zeolites. These are often structural analogues of the aluminosilicate zeolites. Additionally, more recently, other zeolite-like materials, such as metal organic frameworks (ZMOFs) and zeolitic imidazolate frameworks (ZIFs), with topologies similar to that of zeolites, have also been developed. In this document, hereinafter, the term "zeolite" will be used to include all of these zeolite-like materials, as well.

Zeolites are synthesized from a reaction mixture, generally, by means of hydrothermal crystallization, and in some cases by solvothermal crystallization, where said reaction mixture is prepared by mixing suitable proportions of required reactants in order to obtain the desired type of zeolite. While this mixture is being heated, zeolite crystal nuclei are formed within definite periods of time, following which said crystals start to grow. In the presence of a substrate in the medium immersed in the reaction mixture, the nuclei/crystals chemically bind to this substrate, depending on the type of the substrate, and form a zeolite coating that is strongly attached thereon. Properties of this coating depend on experimental conditions such as the composition of the reaction mixture used, reaction temperature, time, method of heating the substrate as well as the presence/absence of mixing and circulation. Use of dilute solutions instead of highly viscous gels commonly used in zeolite synthesis greatly improves coating quality.

Zeolite coatings may be useful for various applications related to adsorption, separation, catalysis and ion-exchange. One significant advantage of these coatings is for the systems where rapid heating/cooling of the adsorbent is required. Adsorption heat pumps and adsorption cooling devices requiring the use of relatively thick zeolite coatings are examples of these systems. Use of structured coatings may reduce pressure drop in adsorptive and catalytic applications, and thus may be advantageous in diffusion limited systems. On the other hand, preparation of thin and uniform coatings may allow the preparation of zeolite membranes, which may be used in various separation and purification applications, such as the separation of water and various alcohols by pervaporation or separation of carbon dioxide and methane or oxygen and nitrogen by gas separation. Use of zeolitic membranes in membrane reactors also presents important opportunities.

Since zeolites are metastable materials, a zeolite phase synthesized from a reaction composition may transform into other phases after longer periods of synthesis. This situation impedes the coatings from being sufficiently thick when the conventional single-step synthesis method is utilized for many zeolite phases. In cases where metastable phase transformation does not occur, since composition of the solution changes as the time increases, as a result of the crystallization activity in the reaction solution, preparing a thick coating is still difficult. Repeated syntheses and other multi-step methods that may be used for preparing thick coatings are not practical or economical. Additionally, the coatings prepared by these methods have compact structures that lead to durability problems due to cracks formed in the coatings in applications requiring fast adsorption/desorption.

In the method of direct heating of the substrate by conduction, wherein the substrate is heated by the help of a resistance (one of the state-of-the-art applications), the reaction mixture is kept at a temperature that is lower than the reaction temperature by the help of a water bath. In this manner, phase transformation of the zeolite is delayed for long periods and thus thicker coatings may be obtained when compared with conventional methods. These coatings also have open structure, high diffusion coefficient and relatively higher durability, all of which are necessary for many applications, such as adsorption heat pump and other heating/cooling applications.

There are several articles in the literature related to direct heating of the substrate materials by using the method of heating by conduction: "Erdem-Senatalar, A., Tatlier, M., Urgen, M., "Preparation of Zeolite Coatings by Direct Heating of the Substrates", Microporous and Mesoporous Materials, 32(3), 331-343 (1999)"; "Tatlier, M., Erdem-Senatalar, A., "The Stability of Zeolite Coatings Grown on Metal Supports for Heat Pump Applications", Studies in Surface Science and Catalysis, Vol. 125, Elsevier, Amsterdam, 101-108 (1999)"; "Tatlier, M., Tantekin-Ersolmaz, S. B., Erdem-Senatalar, A., "Diffusivities of Zeolite Coatings", (Proc. 13th International Zeolite Conference, 2001, Montpellier, France), A. Galarneau, F. Di Renzo, F. Fajula, J. Vedrine (ed.), Studies in Surface Science and Catalysis, Vol. 135, Elsevier, Amsterdam, 3249-3256 (2001)"; "Erdem-Senatalar, A., Oner, K., Tatlier, M., "Searching for Clear Solution Compositions by Using the Substrate Heating Method", Studies in Surface Science and Catalysis, Vol. 154 part A-C, 667-670 (2004)"; "Tatlier, M., Erdem-Senatalar, A., "Estimation of the Effective Diffusion Coefficients in Open Zeolite Coatings", Chemical Engineering Journal, 102(3), 209-216 (2004)"; "Tatlier, M. Demir, M., Tokay, B., Erdem-Senatalar, A., Kiwi-Minsker, L., "Substrate Heating Method for Coating Metal Surfaces with High-Silica Zeolites: ZSM-5 Coatings on Stainless Steel Plates". Microporous and Mesoporous Materials, 101(3), 374-380 (2007)"; Schnabel, L., Tatlier, M., Schmidt, F., Erdem-Senatalar, A., "Adsorption Kinetics of Zeolite Coatings Directly Crystallized on Metal Supports for Heat Pump Applications", Applied Thermal Engineering, 30(11/12), 1409-1416 (2010)".

Large heating resistances and complicated reactors are required to coat large surfaces by using the method of direct heating of the substrate by conduction. Additionally, it may take relatively long times to produce relatively thick coatings using this technique.

Prior art document EP 2 820 170 B1 discloses a zeolite coating preparation assembly and method for using the assembly, that makes the preparation of relatively thick coatings in shorter times possible. In this method, the substrate is heated by induction from a distance, and the reaction mixture is circulated continuously throughout the system. As the substrate in the reactor placed near the induction coil is heated, the temperature of the reaction mixture in the reactor also increases to some degree. The reaction mixture is cooled in a water bath after leaving the reactor to suppress synthesis in the bulk of the mixture. This method may provide relatively thick coatings in relatively short synthesis durations. In this technique, flat plates are used as substrates which are heated by the help of a flat induction coil.

However, uniform heating of large substrate surfaces by using flat plate-flat coil combination is not easy. This type of heating may lead to temperature gradients on the substrate and the coatings obtained may not be so uniform and durable, especially for large substrates. Thus, the preparation of thick, stable and uniform zeolite coatings on large surfaces may present difficulties.

International patent document WO 2010 120 738, an application known in the art discloses a method of coating a metal surface with a protective metal coating having a lower melting point. After the surface to be coated is heated up to the melting point of the metal coating in a high frequency induction heater, the molten metal coating is immediately applied on the heated surface. Chinese patent document CN 101 754 508 discloses an induction heater used for coating steel surfaces. The system includes independent induction heaters and on the upper parts thereof copper coils. Water nozzles are provided at the head ends and the tail ends of the induction coils. Said heater has a simple structure and high efficiency. Japanese patent document JP 2006 256 066 discloses a method for coating the surface of a substrate with a resin. During coating, the resin acquires the same shape as the surface and this shape can be maintained. In the contact process used in the method, the material containing a thermoplastic resin is ensured to contact the surface of the conducting substrate, following which the temperature of the substrate surface is increased by means of the induction heater. "Synthesis of a high-permeance NaA zeolite membrane by microwave heating" by Xu X et al., Advanced Materials, vol. 12, no. 3, 195-198 (2000) discloses the formation of a zeolite coating on a substrate through application of a microwave radiation.

### Objects of the Present Invention

Primary objective of the present invention relates to a zeolite coating preparation assembly and operation method by which synthesis process is shortened owing to the heating by induction, thus saving time.

Another objective of the present invention relates to a zeolite coating preparation assembly and operation method, by which material saving is achieved since large heating resistances and complicated reactors are not used, thus proving to be more economical.

Another objective of the present invention relates to a zeolite coating preparation assembly and operation method, in order to prepare a zeolite coating with desired thickness in shorter periods of time compared to the state of the art.

Another objective of the present invention relates to a zeolite coating preparation assembly and operation method wherein the coatings are obtained in a thicker and more stable form by using a more practical and suitable reaction system.

Another objective of the present invention relates to a zeolite coating preparation assembly and operation method wherein reproducibility and mass production is enabled.

Another objective of the present invention relates to a zeolite coating preparation assembly and operation method wherein scalability is ensured, enabling substrate surfaces of various sizes to be coated.

Another objective of the present invention relates to a zeolite coating preparation assembly and operation method wherein uniform heating of the substrate is ensured, thus more durable coatings, especially on larger substrate surfaces are rendered possible.

Another objective of the present invention relates to a zeolite coating preparation assembly and operation method wherein relatively thin and uniform coatings of membrane character are rendered possible.

### Summary of the Present Invention

The present invention proposes a zeolite coating preparation assembly and operation method for said assembly where, heating by induction and circulation of synthesis solution are preserved/inherited as essential features, however it comprises metal substrates with cylindrical shapes instead of planar, flat plates. Said cylindrically shaped metal substrate is situated within a preferably cylindrically shaped reactor, which itself is placed in the center of a cylindrical induction coil.

With this, the usage of various cylindrically shaped metals, including different porous and nonporous metals as well as wire mesh substrates of various pore sizes and wire thicknesses and their combinations, is rendered possible, technical advantage of which over the state-of-the-art is marked by more uniform and thicker, more durable and more diverse coating capability on larger surfaces to a degree unachievable in the state of the art. Thicknesses on the order of hundreds of micrometers are made possible by the technique.

Metal cylindrical wire mesh substrates are optionally used in single-layer or multi-layer configurations in different embodiments; where all the entities in multi-layer configurations are welded to each other to guarantee the continuity of the electrical conduction paths. The continuity of the electrical conduction paths should be guaranteed in any case, including single layer wire mesh substrates. Wire mesh substrates may also be welded on top of non-porous metal tubes to constitute different types of cylindrical substrates.

Next to that, multi-layer cylindrical wire mesh substrates may additionally be prepared using wire meshes of different pore sizes and wire thicknesses as seen fit.

Various physical and chemical treatments, such as surface oxidation at high temperature in air, aluminizing, sputtering, abrasion/sanding, exposure to acidic/basic solutions and solvents, and coating with various chemicals, may be applied to the substrates to improve their surface characteristics prior to being coated, which in turn improves the binding and crystallization and thus the formation of coating on the surface. Further processing may also be applied on the zeolite-coated metal substrates by coating them with a thin polymer layer in order to reinforce coating durability.

According to the present invention, said assembly and method provides an enhanced coating capability, marked with an increased degree of uniformity due to the cylindrical design of the metal substrate enabling a uniform surface temperature distribution, when heated by induction within the cylindrical induction coil. Said cylindrical design of the system further ensures the flow profile of the synthesis solution along the surface of the substrate to be more uniform; another factor improving the uniformity of the coatings and reproducibility of the coating preparation process.

This design of the system also enables to increase the total surface area that can be coated uniformly. Next to this, said substitution of flat metal plates with cylindrical wire mesh substrates and other porous metals in the presence of a circulating synthesis solution within the system greatly improves the stability and durability of the coating. Usage of multi-layer substrates, whether of wire mesh or porous/non-porous metal character enhances the coating thickness as well as durability. Additionally, wire mesh and some porous metal substrates are lighter, providing more practical and portable systems.

Zeolite coatings may be prepared by using various reaction mixtures with molar compositions, such as 70 Na₂O: 1 Al₂O₃: 15 SiO₂: 2100 H₂O and 50 Na₂O: 1 Al₂O₃: 5 SiO₂: 1000 H₂O for obtaining zeolites X and A, respectively. Conditions for a typical zeolite X synthesis may comprise 12 kW power for the induction device, 358 ml/min circulation rate, 65°C cryostat temperature and 8 h duration; and conditions for a typical zeolite A synthesis may comprise 12 kW power for the induction device, 358 ml/min circulation rate, 35°C cryostat temperature and 5 h duration; both cases for a distance of about 1 cm between the induction coil and a double layer metal wire mesh substrate. Coatings of other synthetic zeolites, may be prepared by this method, using suitable reaction mixtures and synthesis conditions.

When porous substrates, whether of wire mesh or porous metal character, are used, particularly in the case where the pore opening size is small, the proposed method wherein the synthesis solution is circulated, may also allow the reproducible production of thin and uniform coatings, which can be used as membranes for various applications. For membrane preparation, synthesis conditions, such as composition, induction power and temperatures, duration, circulation rate, and volume of the circulated solution, should all be adjusted in order to obtain thinner and continuous crystalline coatings of the desired zeolite phase(s).

### Brief Description of the Figures of the Present Invention

Accompanying drawings are given solely for the purpose of exemplifying a system and method by which preparation of zeolite coating is performed, whose advantages over prior art were outlined above and will be explained in brief hereinafter.

The drawing is not meant to delimit the scope of protection as identified in the claims nor should it be referred to alone in an effort to interpret the scope identified in said claims without recourse to the technical disclosure in the description of the present invention.

Fig. 1 demonstrates a schematic view of an embodiment of the zeolite coating preparation assembly system according to the present invention.

### Detailed Description of the Present Invention

1) Feeding tank
2) Valves (group I)
3) Pump
4) Reactor
5) Induction coil
6) Induction device
7) Metal substrate
8) Valves (group II)
9) Vapor expulsion tank
10) Heat exchanger

P) Pipeline
E) Air outlet

The present invention proposes an assembly and method for zeolite coating preparation, for which the essential method is heating by induction of a metal substrate (7) for which an induction device (6) with an induction coil (5) is utilized. The proposed method further implements a cylindrical metal substrate (7) placed concentrically at the center of a preferably cylindrical reactor (4), which in turn is placed at the center of the cylindrical induction coil (5). Wire meshes, porous and nonporous metals of cylindrical shape may be used as substrates.

The design of the zeolite coating preparation assembly is based on zeolite adsorbents being coated via crystallization process on the surfaces of various substrates heated by induction. Objective of the design is to provide a zeolite coating scheme by which; in addition to time and material savings, the ability of coating larger surfaces reproducibly with more uniform, durable and thicker coatings is achieved. Reproducible preparation of continuous and thin coatings that can be used as membranes is also desired.

The present invention devises the changing of the temperature of the circulating synthesis solution leaving the reactor (4) as heated, by means of a heat exchanger (10). In the preferred embodiment of the invention, the heat exchanger (10) is obtained by passing the pipeline (P) through a cryostat. The synthesis solution does not directly contact the material that the cryostat is made of in this case. The pipeline is made of a material that does not affect the chemical composition of the synthesis solution. Extending the pipeline passing through the cryostat, i.e. heat exchanger (10) "enables the synthesis solution to cool down faster due to increased heat transfer area, and enhances the system volume, allowing the use of higher amounts of synthesis solution.

According to the invention a reactor (4) made of a material with a low electrical conductivity is utilized for preventing zeolite formation on the reactor (4) walls and also for preventing the heated reactor (4) from unnecessarily heating up the synthesis solution, which is allowed to flow through the openings at both ends of the reactor (4). Said reactor (4) is further designed to allow a cylindrical metal substrate (7) to be positioned vertically therein.

In the preferred embodiment of the present invention, the synthesis solution is prepared as diluted in order to allow its circulation in the system. Use of synthesis solutions which are clear to the eye may enhance the quality of the coating. Further in the preferred embodiment of the invention, in order to prevent, or at least delay, metastable phase transformations and to enable the preparation of thick coatings, the cryostat temperature is adjusted so as to keep the temperature of the synthesis solution in the reactor (4) at a desired level that is lower than the temperature of the metal substrate (7).

Also, in the preferred embodiment of the invention, it is ensured that the metal substrate (7) is centered inside the reactor (4) and the reactor (4) is centered inside the induction coil (5). Centering of said metal substrate (7) within said reactor (4) is facilitated by specially designed reactor, preferably comprising lids on both ends, whereas the centering of the said reactor (4) within the said induction coil (5) is finely executed as the distance of said metal substrate (7) to the coil (5) greatly affects the temperature to which the substrate surface is heated.

Cylindrically shaped substrate (7), which is electrically conductive and preferably manufactured out of ferromagnetic material, is positioned vertically inside the reactor (4) preferably after being cleaned with suitable methods known in the state of the art. In the case of wire mesh substrates (7), these elements may be welded at the edges to produce a cylindrical form. Two or more layers of wire mesh substrates may also be welded in a cylindrical fashion to produce multi-layered structures, which may be used as substrates (7) in different applications requiring different embodiments. Substrate (7) should be able to stay in a vertically stable position within the reactor (4), so that the accumulation of crystals on the coating, as they form in the reaction mixture and settle to the bottom of the reactor due to gravity, is prevented.

In the preferred embodiment of the invention, a synthesis solution suitable for the type of zeolite coating desired is prepared from suitable reactants. The synthesis solution should be dilute enough to be circulated, if not clear or clear to the eye, which is considered beneficial for coating quality. The composition of said synthesis solution may be adjusted accordingly so that stable and durable zeolite coatings may be prepared for different applications where different zeolite types and thicknesses may be desired.

In the preferred embodiment of the invention, the cylindrical reactor (4) is centrally positioned within a cylindrical coil (5) connected to an induction device (6) and the cylindrical metal substrate (7) is situated in the reactor (4) in a vertical manner, so that it will remain in the magnetic field of the coil (5) when the induction device (6) is fired. The dimensions of the reactor (4) in which the synthesis reaction is carried out, are determined according to the size of the metal substrate (7) to be used and the amount of synthesis solution to be circulated in the neighbourhood of the heated substrate. Said reactor (4) is preferably manufactured out of a non-conducting, insulating material and further possesses openings at both ends to let the synthesis solution flow through. As it may be applicable sometimes, especially for wire mesh and porous substrates (7); in the cases where both inner and outer surfaces of a substrate (7) are desired to be coated, the synthesis solution should be allowed to flow in a manner to contact both of these sides of the substrate (7).

Synthesis solution in the feeding tank (1) is fed to the system through a pump (3). In a preferred embodiment of the invention, initially, when the synthesis solution is being fed to the system shown in Figure 1, valves denoted with numbers 2a, 2c and 8a are open, conversely to which, valves denoted with numbers 2b, 8b and 8c are closed. In said states of valves, the system is fed to full capacity with said synthesis solution, as to leave no space for air in this path.

Due to the flow within the system and increased temperature of the synthesis solution in the reactor as a result of heating of the substrate by induction, vapor and bubbles may form in the solution. In this case, the vapor and bubbles are delivered to the vapor expulsion tank (9) and thus removed from the solution. In the preferred embodiment of the present invention, diameter of said vapor expulsion tank (9) is greater than the diameter of the pipeline (P) delivering the solution. For some experimental conditions, such as relatively low temperatures that do not lead to much vapor formation, and/or larger pipeline diameters leading to low linear velocities, the use of the vapor expulsion tank (9) and in some cases even the air outlets (E2, E3) may not be necessary. As the temperature in the system (especially the reactor exit temperature) gets closer to 100 °C, the vapor expulsion tank (9) and air outlets can become necessary. When the temperature exceeds 100 °C, the whole system, including the pipeline (P) and all connections should be modified to stand high pressures.

When the use of the vapor expulsion tank is the case, in a preferred embodiment of the invention, after the feeding of the system with the synthesis solution to full capacity, valves 8b and 8c are opened while 8a is closed to fill a certain volume of the vapor expulsion tank (9) and the whole of the pipeline (P) between the vapor expulsion tank (9) and valve 8c.

Next level of the procedure in the disclosed invention involves the circulation of the synthesis solution within the system. In a preferred embodiment of the invention, this is carried out by opening valve 2b and closing valves 2a and 2c. Valves 8b and 8c are kept open and 8a is kept closed in the cases where vapor expulsion is needed. If vapor expulsion is not found necessary, valve 8b is kept closed, while 8a is kept open. Valve 8c may be kept closed or opened if and when pressure release is desired later during synthesis. Then the temperature of the cryostat (10) is adjusted to the desired value and the induction device (6) is powered.

When induction device (6) is powered, a magnetic field is formed that causes the metal substrate (7) inside the reactor (4) to heat up, which in turn causes surrounding synthesis solution passing through the reactor (4) to heat up to a certain extent as well. Power of the induction device (6), as well as the cryostat temperature and circulation rate, are adjusted to obtain the desired synthesis solution temperatures at the entry and exit of the reactor (4), and the substrate (7) temperature, while the distance between metal substrate (7) and induction coil (5) is set at a predetermined value for the same purpose. Substrate (7) temperature, reactor (4) entry and exit temperatures, circulation rate, reaction mixture composition, as well as the synthesis duration affect the type and purity of zeolite phase, coating thickness and texture of the product obtained.

Heated synthesis solution is cooled back to the temperature at the entry of the reactor (4) with the use of the heat exchanger (10). In the preferred embodiment of the present invention, said heat exchanger (10) is formed via passing the pipeline (P) through a cryostat. Said pipeline (P) is, in the preferred embodiment of the present invention, manufactured from a material chemically inert against said synthesis solution. The pipeline (P) in the cryostat is preferred to have a reasonably long length to provide better cooling, in addition to enabling larger amounts of synthesis solution to be circulated in the system.

According to the invention, synthesis solution exiting the heat exchanger (10) at the desired temperature level is delivered back into the reactor (4) with the aid of the pump (3).

In the preferred embodiment of the present invention, after the desired coating is formed displaying appropriate features, process is terminated, and the system is drained. Substrate (7), now coated with zeolite, is removed from the system, rinsed and dried.

In the preferred embodiment of the present invention, said substrate (7) coated with zeolite, is immersed in a polymer solution (e.g. %3 polyacrylic acid) and dried. In this manner, the zeolite coating becomes further coated with a thin layer of polymer increasing its durability.

In short, the present invention proposes a zeolite coating preparation assembly and method for using the same, where a cylindrically designed metal substrate housed in a preferably cylindrical reactor, and a cylindrical induction coil are used. The substrate is heated by induction and the synthesis solution is circulated between the reactor and a heat exchanger continuously. Single or multi-layer wire meshes as well as porous and non-porous metals of cylindrical shape may be used as substrate. In this system, relatively thick, uniform and durable coatings may be prepared reproducibly in relatively short times on relatively large surfaces.

According to the invention, a zeolite coating assembly for the preparation of durable and versatile coatings, comprising at least one feeding tank (1) providing synthesis solution to be used for coating a substrate surface through induction heating made possible with an induction coil (5) connected to an induction device (6) is proposed.

According to the invention, said coating assembly comprises a reactor (4), made of a material with low electrical conductivity, housed inside said cylindrical induction coil (5).

According to the invention, said coating assembly further comprises a cylindrical metal substrate (7), made of an electrically conductive material, placed inside the reactor (4) for uniform coating.

According to the invention, said cylindrical metal substrate (7) further comprises wire meshes, porous or non-porous metals.

According to the invention, said zeolite coating assembly further comprises a pump (3) which enables circulation of the synthesis solution via a pipeline (P).

According to the invention, said zeolite coating assembly further comprises a heat exchanger (10) for changing the temperature of the circulating synthesis solution leaving the reactor (4) as heated.

In a preferred embodiment of the disclosed invention, said metal substrate (7) is centrally positioned within said reactor (4) housed in the said cylindrical induction coil (5), such that the outer surface of said metal substrate (7) is equidistant from said induction coil (5).

In a preferred embodiment of the disclosed invention, said coating assembly further comprises a cylindrical reactor (4) centrally placed in said cylindrical induction coil (5).

In a preferred embodiment of the disclosed invention, said metal substrate (7) comprises at least two layers.

In a preferred embodiment of the disclosed invention, said metal substrate (7) comprises a wire mesh with welded architecture.

In a preferred embodiment of the disclosed invention, said metal substrate (7) further comprises a double-layer wire mesh with welded architecture.

In a preferred embodiment of the disclosed invention, said heat exchanger (10) comprises a cryostat.

In a preferred embodiment of the disclosed invention, said synthesis solution comprises ingredients with desired proportions to result in solution compositions suitable for the synthesis of desired zeolites including zeolite A and zeolite X, as well as zeolite-like materials such as the silicoaluminophosphate SAPO-34 and the aluminophosphate AIPO-5.

In a preferred embodiment of the disclosed invention, said synthesis solution comprises ingredients with desired proportions to result in compositions suitable for synthesis of a mixture of different zeolites and/or zeolite-like material phases.

In a preferred embodiment of the disclosed invention, said metal substrate (7) comprises a welded multi-layered architecture.

In a preferred embodiment of the disclosed invention, said metal substrate (7) comprises features of wire meshes as well as porous and nonporous metals combined in a welded and multi-layered architecture according to an embodiment.

In a preferred embodiment of the disclosed invention, said metal substrate (7) comprises a single wire mesh, a single porous metal or a single nonporous metal.

In a preferred embodiment of the disclosed invention, said metal substrate (7) is made of a ferromagnetic material in order to enhance the effect of the magnetic field generated by the induction device (6) on coating formation.

In a preferred embodiment of the disclosed invention, a method of coating preparation is proposed.

According to the invention, substrate positioning, where metal substrate (7) is positioned in a centralized and vertical manner within said reactor (4), preferably after being cleaned with suitable methods known in the state of the art, takes place.

According to the invention, reactor positioning, where reactor (4) containing the metal substrate (7) is placed vertically and in a centralized manner within said induction coil (5) for the substrate (7) to be uniformly affected by the magnetic field produced when the induction device (6) is turned on takes place.

According to the invention, solution preparation, where a synthesis solution is prepared with predetermined ingredients to comply with the requirements of the coating and is then placed in a feeding tank (1) takes place.

According to the invention, system filling, where synthesis solution is delivered from the feeding tank (1) to the system, at the chosen rate with the aid of a pump (3) and with the chosen configuration of valves in the system, such that it will pass through the reactor (4) and the heat exchanger (10) replacing any and all air on its path takes place.

According to the invention, adjusting the power of the induction device (6), and the temperature of the heat exchanger (10), in order to provide the desired substrate temperature, and the desired reactor inlet temperature of the synthesis solution that will be heated to a certain extent in the reactor (4) by the heated substrate (7) when the induction device is turned on takes place.

According to the invention, powering the induction device (6), in order to produce magnetic field and thus heat the substrate (7) takes place.

In a preferred embodiment of the disclosed invention, circulation, where the pump (3) continuously delivers the heated synthesis solution to the heat exchanger (10) and the cooled synthesis solution back to the reactor (4), also allowing expulsion of vapor and depressurization of the system, if and when necessary, with the aid of chosen configuration of valves, takes place.

According to the invention, synthesis, where the desired coating with desired properties, is prepared on the substrate (7) under previously chosen conditions with continuous circulation for the required period, takes place.

According to the invention, recovery, where the process is terminated, and the zeolite coated substrate (7) is removed from the system, and is rinsed and dried, takes place.

In a preferred embodiment of the disclosed invention, when vapor expulsion is necessary, after the said system filling step, additional synthesis solution is admitted into the system by using the chosen valves, in order to be able to expel later, the vapor and bubbles produced as a result of induction heating, with the aid of the vapor expulsion tank (9).

In a preferred embodiment of the disclosed invention, said substrate positioning step of said method is preceded by a treatment step comprising treatment of said metal substrate (7) using various physical and/or chemical methods selected from a group including surface oxidation at high temperature in air, aluminizing, sputtering, abrasion/sanding, exposure to acidic/basic solutions and solvents, and coating with various chemicals.

In a preferred embodiment of the disclosed invention, said zeolite-coated substrate recovery step of said method is succeeded by a treatment step comprising the treatment of said coated metal substrate (7) using various chemicals, such as polymeric solutions.

In a preferred embodiment of the disclosed invention, a membrane is manufactured.

## Claims

1. A zeolite coating assembly for the preparation of durable and versatile coatings, comprising at least one feeding tank (1) providing synthesis solution to be used for coating a substrate surface through induction heating via an induction coil (5) connected to an induction device (6);
said zeolite coating assembly further comprises a pump (3) which enables circulation of the synthesis solution via a pipeline (P);
said zeolite coating assembly further comprises a heat exchanger (10) for changing the temperature of the circulating synthesis solution leaving the reactor (4) as heated;
**characterized in that** said coating assembly comprises a reactor, made of a material with low electrical conductivity, housed inside said cylindrical induction coil;said coating assembly further comprises a cylindrical metal substrate, made of an electrically conductive material, placed inside the reactor;said cylindrical metal substrate further comprises wire meshes, porous or non-porous metals.

2. A zeolite coating assembly, as set forth in Claim 1 **characterized in that** said metal substrate (7) is centrally positioned within said reactor (4) housed in the said cylindrical induction coil (5), such that the outer surface of said metal substrate (7) is equidistant from said induction coil (5).

3. A zeolite coating assembly, as set forth in Claim 1 **characterized in that** said reactor (4) centrally placed in said cylindrical induction coil (5) is cylindrical.

4. A zeolite coating assembly, as set forth in Claim 1 **characterized in that** said metal substrate (7) comprises at least one layer.

5. A zeolite coating assembly, as set forth in Claim 4 **characterized in that** said metal substrate (7) comprises a wire mesh or a double-layer wire mesh with welded architecture.

6. A zeolite coating assembly, as set forth in Claims 2, 4 and 5 **characterized in that** said metal substrate (7) comprises a welded multi-layered architecture.

7. A zeolite coating assembly, as set forth in Claim 6 **characterized in that** said metal substrate (7) comprises a combination of wire meshes, porous and nonporous metals in a welded and multi-layered architecture according to an embodiment.

8. A zeolite coating assembly, as set forth in Claim 6 **characterized in that** said metal substrate (7) comprises a single wire mesh, a single porous metal or a single nonporous metal.

9. A zeolite coating assembly, as set forth in Claim 1 **characterized in that** said metal substrate (7) is made of a ferromagnetic material in order to enhance the effect of the magnetic field generated by the induction device (6) on coating formation.

10. A zeolite coating assembly, as set forth in Claim 1 **characterized in that** said heat exchanger (10) comprises a cryostat.

11. A zeolite coating assembly, as set forth in Claim 1 **characterized in that** said synthesis solution comprises ingredients with desired proportions to result in solution compositions suitable for the synthesis of desired zeolites including zeolite A and zeolite X, zeolite-like materials, such as the silicoaluminophosphate SAPO-34 and the aluminophosphate AIPO-5, as well as mixtures of said different zeolites and/or zeolite-like materials.

12. A method of coating preparation **characterized in that** said method comprises steps of;
substrate positioning, where a cylindrical metal substrate (7) is positioned in a centralized and vertical manner within a reactor (4) preferably after being cleaned with suitable methods known in the state of the art;
reactor positioning, where reactor (4) containing the metal substrate (7) is placed vertically and in a centralized manner within a cylindrical induction coil (5) for the substrate (7) to be uniformly affected by the magnetic field produced when an induction device (6) is turned on;
solution preparation, where a synthesis solution is prepared with predetermined ingredients to comply with the requirements of the coating and is then placed in a feeding tank (1);
system filling, where synthesis solution is delivered from the feeding tank (1) to the system, at the chosen rate with the aid of a pump (3) and with the chosen configuration of valves in the system, such that it will pass through the reactor (4) and a heat exchanger (10) replacing any and all air on its path;
adjusting the power of the induction device (6), and the temperature of the heat exchanger (10), in order to provide the desired substrate temperature, and the desired reactor inlet temperature of the synthesis solution that will be heated to a certain extent in the reactor (4) by the heated substrate (7) when the induction device is turned on;
powering the induction device (6), in order to produce magnetic field and thus heat the substrate (7);
circulation, where the pump (3) continuously delivers the heated synthesis solution to the heat exchanger (10) and the cooled synthesis solution back to the reactor (4), also allowing expulsion of vapor and depressurization of the system, if and when necessary, with the aid of chosen configuration of valves;
synthesis, where the desired coating with desired properties, is prepared on the substrate (7) under previously chosen conditions with continuous circulation for the required period; and,
recovery, where the process is terminated, and the zeolite coated substrate (7) is removed from the system, rinsed and dried.

13. A method of coating preparation as set forth in Claim 12, **characterized in that,** when vapor expulsion is necessary, after the said system filling step, additional synthesis solution is admitted into the system by using the chosen valves, in order to be able to expel later, the vapor and bubbles produced as a result of induction heating, with the aid of the vapor expulsion tank (9).

14. A method of coating preparation as set forth in Claim 12, **characterized in that** said substrate positioning step of said method is preceded by a treatment step comprising treatment of said metal substrate (7) using various physical and/or chemical methods selected from a group including surface oxidation at high temperature in air, aluminizing, sputtering, abrasion/sanding, exposure to acidic/basic solutions and solvents, and coating with various chemicals.

15. A method of coating preparation as set forth in Claim 12, **characterized in that** said zeolite-coated substrate recovery step of said method is succeeded by a treatment step comprising the treatment of said coated metal substrate (7) using various chemicals, such as polymeric solutions.

## Patentansprüche

1. Zeolith-Beschichtungsanordnung zur Herstellung von dauerhaften und vielseitigen Beschichtungen, die mindestens einen Speisebehälter (1) aufweist, der eine, zur Beschichtung einer Substratoberfläche durch Induktionserwärmung zu verwendende Syntheselösung bereitstellt, wobei die Induktionserwärmung mit einer an eine Induktionsvorrichtung (6) verbundene Induktionsspule (5) ermöglicht wird,
wobei die Zeolith-Beschichtungsanordnung außerdem eine Pumpe (3) aufweist, die die Zirkulation der Syntheselösung über eine Rohrleitung (P) ermöglicht;
wobei die Zeolith-Beschichtungsanordnung ferner, zur Änderung der Temperatur der zirkulierenden, den Reaktor (4) im erhitzten Zustand verlassenden Syntheselösung einen Wärmetauscher (10) aufweist,
**dadurch gekennzeichnet, dass** die Beschichtungsanordnung einen Reaktor aus einem Material mit niedriger elektrischer Leitfähigkeit aufweist, der im Inneren der zylindrischen Induktionsspule untergebracht ist; die Beschichtungsanordnung ferner ein zylindrisches Metallsubstrat aus einem elektrisch leitenden Material aufweist, das im Inneren des Reaktors angeordnet ist; das zylindrische Metallsubstrat ferner Drahtgitter, poröse oder nicht poröse Metalle aufweist.

2. Zeolith-Beschichtungsanordnung gemäß Anspruch 1, **dadurch gekennzeichnet, dass** das Metallsubstrat (7) innerhalb des in der zylindrischen Induktionsspule untergebrachten Reaktors (4) mittig positioniert ist, so dass die Außenfläche des Metallsubstrats (7) von der Induktionsspule (5) gleich weit entfernt ist.

3. Zeolith-Beschichtungsanordnung gemäß Anspruch 1, **dadurch gekennzeichnet, dass** der in der zylindrischen Induktionsspule (5) mittig platzierter Reaktor (4) zylindrisch ist.

4. Zeolith-Beschichtungsanordnung gemäß Anspruch 1, **dadurch gekennzeichnet, dass** das Metallsubstrat (7) mindestens eine Schicht aufweist.

5. Zeolith-Beschichtungsanordnung gemäß Anspruch 4, **dadurch gekennzeichnet, dass** das Metallsubstrat (7) ein Drahtgitter oder ein doppelschichtiges Drahtgitter mit geschweißter Architektur aufweist.

6. Zeolith-Beschichtungsanordnung gemäß Anspruch 2, 4 und 5, **dadurch gekennzeichnet, dass** das Metallsubstrat (7) eine geschweißte mehrschichtige Architektur aufweist.

7. Zeolith-Beschichtungsanordnung gemäß Anspruch 6, **dadurch gekennzeichnet, dass** das Metallsubstrat (7) eine Kombination von Drahtgittern, porösen und nicht porösen Metallen in einer geschweißten und mehrschichtigen Architektur gemäß einer Ausführungsform aufweist.

8. Zeolith-Beschichtungsanordnung gemäß Anspruch 6, **dadurch gekennzeichnet, dass** das Metallsubstrat (7) ein einzelnes Drahtgitter, ein einzelnes poröses Metall oder ein einzelnes nichtporöses Metall aufweist.

9. Zeolith-Beschichtungsanordnung gemäß Anspruch 1, **dadurch gekennzeichnet, dass** das Metallsubstrat (7) aus einem ferromagnetischen Material hergestellt ist, um die Wirkung des von der Induktionsvorrichtung (6) erzeugten Magnetfeldes auf die Beschichtungsbildung zu verstärken.

10. Zeolith-Beschichtungsanordnung gemäß Anspruch 1, **dadurch gekennzeichnet, dass** der Wärmetauscher (10) einen Kryostaten aufweist.

11. Zeolith-Beschichtungsanordnung gemäß Anspruch 1, **dadurch gekennzeichnet, dass** die Syntheselösung Bestandteile mit gewünschten Anteilen aufweist, um Lösungszusammensetzungen zu ergeben, die für die Synthese von gewünschten Zeolithen, einschließlich Zeolith A und Zeolith X, Zeolith ähnlichen Materialien, wie dem Silica-Alumino-Phosphat SAPO-34 und dem Alumino-Phosphat AlPO-5, sowie von Mischungen der verschiedenen Zeolithe und/oder Zeolith ähnlichen Materialien geeignet sind.

12. Verfahren zur Herstellung einer Beschichtung, **dadurch gekennzeichnet, dass** das Verfahren die folgenden Schritte umfasst;
das Positionieren des Substrats, bei dem ein zylindrisches Metallsubstrat (7) zentralisiert und vertikal in einem Reaktor (4) positioniert wird, vorzugsweise nachdem es mit geeigneten, im Stand der Technik bekannten Methoden gereinigt wurde;
das Positionieren des Reaktors, bei dem der Reaktor (4) der das Metallsubstrat (7) enthält vertikal und zentralisiert in einer zylindrischen Induktionsspule (5) platziert wird, damit das Substrat (7) gleichmäßig von dem Magnetfeld beeinflusst wird, das beim Einschalten einer Induktionsvorrichtung (6) erzeugt wird;
das Zubereiten der Lösung, bei dem eine Syntheselösung mit vorbestimmten Bestandteilen entsprechend den Anforderungen der Beschichtung zubereitet und dann in einen Speisebehälter (1) gegeben wird;
das Befüllen des Systems, bei dem die Syntheselösung aus dem Speisebehälter (1) mit Hilfe einer Pumpe (3) und der ausgewählten Konfiguration der Ventile im System mit einer ausgewählten Geschwindigkeit in das System geleitet wird, so dass sie den Reaktor (4) und einen Wärmetauscher (10) durchläuft und dabei die gesamte Luft auf ihrem Weg verdrängt;
das Einstellen der Leistung der Induktionsvorrichtung (6) und der Temperatur des Wärmetauschers (10), um eine gewünschte Substrattemperatur und eine gewünschte Reaktoreinlasstemperatur der Syntheselösung bereitzustellen, die im Reaktor (4) durch das erhitzte Substrat (7) bis zu einem gewissen Grad erhitzt wird, wenn die Induktionsvorrichtung eingeschaltet ist;
das Versorgen der Induktionsvorrichtung (6) mit Strom, um ein Magnetfeld zu erzeugen und so das Substrat (7) zu erwärmen;
das Zirkulieren, bei dem die Pumpe (3) kontinuierlich die erwärmte Syntheselösung zum Wärmetauscher (10) und die abgekühlte Syntheselösung zurück zum Reaktor (4) befördert, wobei mit Hilfe der gewählten Konfiguration der Ventile auch das Ausstoßen des Dampfes und die Druckentlastung des Systems ermöglicht wird;
die Synthese, bei der die gewünschte Beschichtung mit den gewünschten Eigenschaften auf dem Substrat (7) unter vorher gewählten Bedingungen mit der kontinuierlichen Zirkulation für den erforderlichen Zeitraum hergestellt wird; und,
die Rückgewinnung, bei der der Prozess beendet und das Zeolith beschichtete Substrat (7) aus dem System entfernt, gespült und getrocknet wird.

13. Verfahren zur Herstellung einer Beschichtung gemäß Anspruch 12, **dadurch gekennzeichnet, dass** wenn nach dem Schritt des Befüllens des Systems ein Dampfausstoß erforderlich ist, unter Verwendung von ausgewählten Ventilen zusätzliche Syntheselösung in das System eingelassen wird, um später den Dampf und die Blasen, die als Ergebnis der Induktionserwärmung erzeugt werden, mit Hilfe des Dampfausstoßbehälters (9) ausstoßen zu können.

14. Verfahren zur Herstellung einer Beschichtung gemäß Anspruch 12, **dadurch gekennzeichnet, dass** dem Schritt des Positionierens des Substrats in dem Verfahren ein Schritt des Behandelns vorausgeht, der das Behandeln des Metallsubstrats (7) unter Verwendung verschiedener physikalischer und/oder chemischer Verfahren umfasst, die aus einer Gruppe ausgewählt ist, umfassend: das Oxidieren der Oberfläche in der Luft bei hoher Temperatur, Aluminieren, Sputtern, Abschleifen/Schmirgeln, Aussetzen zur sauren/basischen Lösungen und Lösungsmitteln und Beschichten mit verschiedenen Chemikalien.

15. Verfahren zur Herstellung einer Beschichtung gemäß Anspruch 12, **dadurch gekennzeichnet, dass** auf den Schritt der Rückgewinnung des Zeolith beschichteten Substrats in dem Verfahren ein Schritt des Behandelns folgt, umfassend das Behandeln des beschichteten Metallsubstrats (7) unter Verwendung verschiedener Chemikalien, wie z.B. polymerer Lösungen.

## Revendications

1. Assemblage de revêtement de zéolithe pour la préparation de revêtements durables et polyvalents, comprenant au moins un réservoir d'alimentation (1) fournissant une solution de synthèse à utiliser pour le revêtement d'une surface de substrat par chauffage par induction rendu possible par une bobine d'induction (5) reliée à un dispositif d'induction (6).
ledit assemblage de revêtement de zéolithe comprenant en outre une pompe (3) qui permet la circulation de la solution de synthèse via un pipeline (P) ;
ledit assemblage de revêtement de zéolithe comprenant en outre un échangeur de chaleur (10) pour modifier la température de la solution de synthèse circulante qui quitte le réacteur (4) après avoir été chauffée,
**caractérisé en ce que** l'assemblage de revêtement comprend un réacteur, constitué d'un matériau à faible conductivité électrique, logé à l'intérieur de la bobine d'induction cylindrique; l'assemblage de revêtement comprenant en outre un substrat métallique cylindrique, constitué d'un matériau conducteur d'électricité, placé à l'intérieur du réacteur; ledit substrat métallique cylindrique comprenant en outre des grillages métalliques, des métaux poreux ou non poreux.

2. Assemblage de revêtement de zéolithe selon la revendication 1, **caractérisé en ce que** ledit substrat métallique (7) est positionné au centre dudit réacteur (4) logé dans ladite bobine d'induction cylindrique (5), de telle sorte que la surface extérieure dudit substrat métallique (7) est équidistante de ladite bobine d'induction (5).

3. Assemblage de revêtement de zéolithe selon la revendication 1, **caractérisé en ce que** le réacteur (4) placé au centre de la bobine d'induction cylindrique (5) est cylindrique.

4. Assemblage de revêtement de zéolithe selon la revendication 1, **caractérisé en ce que** le substrat métallique (7) comprend au moins une couche.

5. Assemblage de revêtement de zéolithe selon la revendication 4, **caractérisé en ce que** le substrat métallique (7) comprend un grillage métallique ou un grillage métallique à double couche avec une architecture soudée.

6. Assemblage de revêtement de zéolithe selon les revendications 2, 4 et 5, **caractérisé en ce que** le substrat métallique (7) comprend une architecture multicouche soudée.

7. Assemblage de revêtement de zéolithe, selon la revendication 6, **caractérisé en ce que** ledit substrat métallique (7) comprend une combinaison de grillages métalliques, de métaux poreux et non poreux dans une architecture soudée et multicouche selon un mode de réalisation.

8. Assemblage de revêtement de zéolithe selon la revendication 6, **caractérisé en ce que** le substrat métallique (7) comprend un seul grillage métallique, un seul métal poreux ou un seul métal non poreux.

9. Assemblage de revêtement de zéolithe selon la revendication 1, **caractérisé en ce que** le substrat métallique (7) est constitué d'un matériau ferromagnétique afin de renforcer l'effet du champ magnétique généré par le dispositif d'induction (6) sur la formation du revêtement.

10. Assemblage de revêtement de zéolithe selon la revendication 1, **caractérisé en ce que** l'échangeur de chaleur (10) comprend un cryostat.

11. Assemblage de revêtement de zéolithe selon la revendication 1, **caractérisé en ce que** ladite solution de synthèse comprend des ingrédients dans les proportions souhaitées afin d'obtenir des compositions de solution adaptées à la synthèse des zéolithes souhaitées, y compris la zéolithe A et la zéolithe X, des matériaux de type zéolithe tels que le silice-aluminophosphate SAPO-34 et l'aluminophosphate AlPO-5, ainsi que des mélanges de ces différentes zéolithes et/ou de matériaux de type zéolithe.

12. Méthode de préparation de revêtement **caractérisée en ce que** ladite méthode comprend les étapes suivantes;
le positionnement du substrat, où un substrat métallique cylindrique (7) est positionné verticalement et de manière centralisée dans un réacteur (4), de préférence après avoir été nettoyé à l'aide de méthodes appropriées connues dans l'état de l'art;
le positionnement du réacteur, où le réacteur (4) contenant le substrat métallique (7) est placé verticalement et de manière centralisée dans une bobine d'induction cylindrique (5) pour que le substrat (7) soit uniformément affecté par le champ magnétique produit lorsqu'un dispositif d'induction (6) est mis en marche;
la préparation de la solution, où une solution de synthèse est préparée avec des ingrédients prédéterminés pour répondre aux exigences du revêtement et est ensuite placée dans un réservoir d'alimentation (1);
le remplissage du système, où la solution de synthèse est acheminée du réservoir d'alimentation (1) vers le système, au débit choisi, à l'aide d'une pompe (3) et avec la configuration choisie des vannes dans le système, de sorte qu'elle traverse le réacteur (4) et un échangeur de chaleur (10) en remplaçant tout l'air qui se trouve sur son chemin; régler la puissance du dispositif d'induction (6) et la température de l'échangeur de chaleur (10) afin d'obtenir la température souhaitée du substrat et la température souhaitée à l'entrée du réacteur de la solution de synthèse qui sera chauffée dans une certaine mesure dans le réacteur (4) par le substrat chauffé (7) lorsque le dispositif d'induction est mis en marche ;
l'alimentation du dispositif d'induction (6), afin de produire un champ magnétique et donc de chauffer le substrat (7) ;
la circulation, où la pompe (3) refoule en continu la solution de synthèse chauffée vers l'échangeur de chaleur (10) et la solution de synthèse refroidie vers le réacteur (4), permettant également l'expulsion de la vapeur et la dépressurisation du système, à l'aide d'une configuration choisie de vannes ;
la synthèse, où le revêtement souhaité avec les propriétés souhaitées, est préparé sur le substrat (7) dans des conditions préalablement choisies avec une circulation continue pendant la période requise ; et,
la récupération, où le procédé est terminé et le substrat revêtu de zéolithe (7) est retiré du système, rincé et séché.

13. Méthode de préparation de revêtement selon la revendication 12, **caractérisée en ce que**, lorsque l'expulsion de la vapeur est nécessaire, après ladite étape de remplissage du système une solution de synthèse supplémentaire est admise dans le système à l'aide des vannes choisies, afin de pouvoir expulser ultérieurement la vapeur et les bulles produites à la suite du chauffage par induction, à l'aide du réservoir d'expulsion de la vapeur (9).

14. Méthode de préparation de revêtement selon la revendication 12, **caractérisée en ce que** l'étape de positionnement du substrat de ladite méthode est précédée d'une étape de traitement comprenant le traitement dudit substrat métallique (7) à l'aide de diverses méthodes physiques et/ou chimiques choisies dans un groupe comprenant l'oxydation de surface à haute température dans l'air, l'aluminisation, la pulvérisation, l'abrasion/le sablage, l'exposition à des solutions acides/bases et à des solvants, et le revêtement à l'aide de divers produits chimiques.

15. Méthode de préparation de revêtement selon la revendication 12, **caractérisée en ce que** l'étape de récupération du substrat revêtu de zéolithe de ladite méthode est suivie d'une étape de traitement comprenant le traitement dudit substrat métallique revêtu (7) à l'aide de divers produits chimiques, tels que des solutions polymériques.
